

## UNITED STATES PATENT OFFICE

2,582,086

COMPOSITION FOR CARROTING FUR  
AND THE LIKE

Harold H. Tucker, Scarsdale, N. Y., and Raymond J. Trimpert, Newtown, Conn., assignors to The Frank H. Lee Company, Danbury, Conn.

No Drawing. Application December 23, 1949,  
Serial No. 134,860

5 Claims. (Cl. 8—112)

1

Our invention relates to the treatment of fur and similar animal fibers to improve the felting qualities, otherwise known as "carrotting," and more particularly to a composition of matter adapted to be employed in such treatment.

To produce a material such as felt from fur and the like, it is first necessary to treat the fur to promote ease and rapidity of felting, and to acquire a high strength product. A preliminary chemical treatment, known as "carrotting," is generally used, and it involves applying a relatively strong oxidizing and/or hydrolyzing aqueous solution to the fur before it is sheared from the skin. The solution may be applied by any suitable means, as by brushing, and the pelts are either air-dried or oven-dried before shearing. The fur is then graded, blended, and, by a process of treatment with hot water and pressure applications, is formed into a felt whereby fibers become tightly interlocked and compactly associated with one another.

The chemical reagents have the faculty of rendering this process of felting more thorough and efficient, the mechanics of which have never been explained satisfactorily. Nevertheless, perhaps the most successful carrot is an acid solution of a mercury salt, but being toxic it may not be used because of its harm to the workmen. Consequently, many substitutes have been developed, and these generally are strong solutions of oxidizing and hydrolyzing reagents such as mineral acids, organic acids, salts of these acids, peroxides, and the like. A carrotting solution by its very nature damages the fur, and so the problem in selecting any composition for this purpose is to provide sufficient treatment for successful felting without at the same time destroying the strength of the fibers. Accordingly, a common difficulty arises from the use of these mercury carrot substitutes because they ordinarily must be relatively strong to render the fur feltable, with the result that fibers are inordinately damaged. Indeed these substitutes have a high specific gravity, normally above 6° Baumé, and generally about 8° Baumé.

It is accordingly among the objects of our invention to provide a carrotting solution which renders fur feltable without deleteriously altering the strength and wearing qualities of the final product.

A further object is to provide a successful and practical carrotting solution with a low specific gravity, for example, in the range of 3°-5° Baumé. Another object is to use a carrotting solution composed of inexpensive reagents where-

2

ever possible, and to employ only small percentages of expensive ingredients so that the cost of carrotting is maintained within commercially acceptable limits. A still further object is to provide a carrotting solution which is not toxic under ordinary conditions of its use.

Various changes in and departures from the embodiment of our carrotting composition may be made as the same is hereinafter exemplified, all within the scope of our generic invention, it being understood that the matter set forth is submitted as illustrative and not in a limiting sense.

Our new and improved composition is an aqueous solution of reagents which are well known for their oxidizing and/or hydrolyzing characteristics, but which are combined in such proportions and with certain other ingredients that a far weaker solution than hitherto thought possible can be used to carrot fur for successful felting. Being relatively weak, however, the solution does not unduly damage the fur so that a strong, high quality felt is produced.

The preferred embodiment of our carrotting solution contains a small percentage of one or more strong or moderately strong acids, such as hydrochloric and nitric, together with an oxidizing agent such as hydrogen peroxide, and a small amount of ethyl alcohol, to produce a solution with a specific gravity in the order of 3°-5° Baumé. Such weak solutions are incapable of carrotting the fur within practical limits, but we have discovered that the addition of a small amount of either phosphotungstic acid or phosphomolybdic acid renders them highly satisfactory for this purpose.

This preferred solution contains nitric acid in the order of 1-3% together with 0-1.5% hydrochloric acid, though nitric acid may be used alone with equivalent results. These proportions are computed as percentages of  $\text{HNO}_3$  and  $\text{HCl}$ , respectively, in the entire weight of liquid. In addition to the acid, a small amount of strong oxidizing agent, such as 3-5% by weight of hydrogen peroxide is used (computed as  $\text{H}_2\text{O}_2$ ), together with 0.3-1% by weight of ethyl alcohol (computed as  $\text{C}_2\text{H}_5\text{OH}$ ). The specific gravity of the final mixture is about 3° Baumé.

Carrotting with this solution is not successful, but when 0.1-0.4% by weight of either phosphotungstic acid or phosphomolybdic acid or a combination of the two is added, a high strength, good quality felt can be produced. The specific gravity of the final solution is preferably within

the range of 3-5° Baumé and consequently little damage to the fur is encountered as with other known solutions ranging from 6-8° Baumé and upwards.

Considering the infinitesimal amounts of the phosphotungstic or phosphomolybdic acids which are employed, it is most probable that a catalytic action is encountered, whereby the reagents are utilized more efficiently. The weak solution in itself is not satisfactory and therefore it would seem that such a small proportion of the phosphotungstic and phosphomolybdic acids would hardly fulfill the need for more reaction to overcome such deficiency. Yet the addition of this small amount of phosphotungstic or phosphomolybdic acid does have this remarkable effect. It should be understood, however, that we do not desire to be restricted in our invention to any particular theory, it being sufficient that the result herein described is accomplished.

Several tests have been conducted to determine composition limits and substitutes for our preferred carotting solution. Considering the acids, those which are strong or moderately strong are the most useful, and their content should be kept quite low, commensurate with good results, and indeed it should never be necessary to use over 4.5% by weight. Highly satisfactory carrots are obtained by the use of the combination of nitric acid and hydrochloric acid, or of nitric acid alone; however hydrochloric acid by itself appears inferior.

The strong oxidizing agent, hydrogen peroxide, supplements the action of the acid in treating the animal fibers, but its concentration is maintained within the limits of 3-5% to avoid undue damage which weakens the final felt.

A small amount of organic solvent, such as ethyl alcohol, is beneficial in causing the fibers to wet more readily, and its cleansing properties are generally thought to cause more uniformity of treatment.

Since the carotting reaction by its very nature causes damage to fur fibers, the primary object in developing any satisfactory composition for this purpose is to balance the adverse factors so that the best combination of quality and strength of felt is obtained. Ofttimes a good quality felt, as judged by the feel, may be produced from fur which is rather severely damaged, but the final product will have poor wearing properties and will prove to be weak when judged by certain physical tests such as tensile strength and flexing value determinations. Conversely, when damage is avoided it is impossible to obtain a good, strong, tight felt. Either the felting rate is so slow that an appreciable quantity of fur is lost while felting, or felting stops before final size is reached, after which further work merely increases the size of the hat body.

The limits of 0.1-0.4% for phosphotungstic or phosphomolybdic acids are critical in providing the optimum combination of strong, good quality felt. These were determined by preparing a series of basic carotting solutions containing 1.54% HNO<sub>3</sub>, 0.73% HCl, 0.4% C<sub>2</sub>H<sub>5</sub>OH, 3.3% H<sub>2</sub>O<sub>2</sub> and phosphotungstic acid varying in amounts from 0 to 1.6%. These various solutions were then used to carrot rabbit fur, and felt hats were made by usual commercial practice.

The flexing test is perhaps the most significant physical test for evaluating damage to fur felt, whether resulting from carotting or subsequent manufacturing processes such as dyeing. A flexing machine is commercially available for this

test, and its use on fur felt hats is well known in the art. In this test a sample of felt one-half inch wide and six inches long is held in a flexing machine under tension of two and one-half pounds and is subjected to repeated bendings at the rate of 110 flexes per minute until it breaks. The flex value is the average number of flexes required to break eight samples cut from different portions of the hat so that all sections thereof may be tested.

A felt made from fur carotted with the basic solution without any phosphotungstic acid has a high flex value because the solution is weak and does little damage. As mentioned above, this basic solution comprises 1.54% HNO<sub>3</sub>, 0.73% HCl, 0.4% C<sub>2</sub>H<sub>5</sub>OH and 3.3% H<sub>2</sub>O<sub>2</sub>, balance water. However, the felt is loose and soft as judged by its feel, and the time and number of operations required to produce the felt are inordinately high.

20 The flex values of the felts become progressively lower as the amount of phosphotungstic acid in the carotting solution is increased, and when 0.4% is exceeded the quality and felting rates are erratic and the felts are of such poor strength as not to be useful commercially. Consequently, the practical range is between 0.1-0.4% phosphotungstic acid in the carotting solution having a specific gravity of only 3-5° Baumé. Phosphomolybdic acid may be substituted in like amounts to obtain equivalent results.

The phosphotungstic acid employed in the above tests has the formula P<sub>2</sub>O<sub>5</sub>.24WO<sub>3</sub>.44H<sub>2</sub>O, and the phosphomolybdic acid has the formula 20MoO<sub>3</sub>.2H<sub>3</sub>PO<sub>4</sub>.48H<sub>2</sub>O.

35 The cost of these acids is very high and for commercial use it is usually advisable to limit its concentration to about 0.2%, since the results appear equally satisfactory throughout the recommended range.

40 As many possible embodiments may be made of the above invention and as many changes might be made in the composition above set forth, it is to be understood that all matter hereinbefore set forth is to be interpreted as illustrative and not in a limiting sense.

What is claimed is:

1. As a composition of matter for the carotting of fur or the like, an aqueous carotting solution containing a non-hydrolyzing oxidizing agent, a volatile hydrolyzing acid, and an acid of the group consisting of phosphotungstic acid and phosphomolybdic acid as a catalyst, said solution having the proportions of 1.0-4.5% by weight said hydrolyzing acid, 3-5% by weight said oxidizing agent, and 0.1-0.4% by weight of said latter acid or acids.

2. An aqueous carotting solution for treating fur and the like containing 3-5% by weight hydrogen peroxide, 1-3% by weight nitric acid, and as a catalyst 0.1-0.4% by weight phosphotungstic acid, the specific gravity of said solution being between 3-5° Baumé.

3. An aqueous carotting solution for treating fur and the like containing 3-5% by weight hydrogen peroxide, 1-3% by weight nitric acid, and as a catalyst 0.1-0.4% by weight phosphomolybdic acid, the specific gravity of said solution being between 3-5° Baumé.

4. An aqueous carotting solution for treating fur and the like containing 1-3% by weight nitric acid, hydrochloric acid not to exceed 1.5% by weight, 3-5% by weight hydrogen peroxide, as a catalyst 0.1-0.4% by weight phosphotungstic

acid, and 0.3-1.0% by weight ethyl alcohol, the specific gravity of said solution being between 3-5° Baumé.

5. An aqueous carotting solution for treating fur and the like, containing 3-5% by weight hydrogen peroxide, 1-3% by weight nitric acid, 0.3-1% by weight ethyl alcohol, and as a catalyst 0.1-0.4% by weight phosphotungstic acid, the specific gravity of said solution being between 3°-5° Baumé.

HAROLD H. TUCKER.  
RAYMOND J. TRIMPERT.

## REFERENCES CITED

The following references are of record in the file of this patent:

## UNITED STATES PATENTS

| Number       | Name           | Date          |
|--------------|----------------|---------------|
| 1,710,565    | Bohm           | Apr. 23, 1929 |
| 2,048,645    | Fabian         | July 21, 1936 |
| 2,087,854    | Fabian         | July 20, 1937 |
| 2,169,997    | Fabian         | Aug. 22, 1939 |
| 2,181,884    | Giuliano       | Dec. 5, 1939  |
| 2,242,668    | Dolid          | May 20, 1941  |
| 2,330,813    | Donner         | Oct. 5, 1943  |
| 10 2,411,725 | Hodshon et al. | Nov. 26, 1946 |

## FOREIGN PATENTS

| Number     | Country                                         | Date          |
|------------|-------------------------------------------------|---------------|
| 15 323,944 | Great Britain                                   | Jan. 16, 1930 |
| 441,619    | Canada                                          | 1947          |
|            | (Through J. Am. Leather Chem. Assn., Nov. 1947. |               |
|            | page 588)                                       |               |
| 803,872    | France                                          | Oct. 10, 1936 |